

April 25, 1961

E. ALBERS-SCHOENBERG

2,981,690

FERRITES WITH SQUARE HYSTERESIS LOOPS

Filed June 18, 1957



INVENTOR  
ERNST ALBERS-SCHOENBERG

BY  
Greene, Penick & Draper

ATTORNEYS

2,981,690

## FERRITES WITH SQUARE HYSTERESIS LOOPS

Ernst Albers-Schoenberg, Metuchen, N.J., assignor to Steatite Research Corporation, Keasbey, N.J., a corporation of Delaware

Filed June 18, 1957, Ser. No. 666,456

5 Claims. (Cl. 252—62.5)

This invention relates to fired ferrite compositions which have square or rectangular hysteresis loops.

Square-hysteresis-loop ferrites have become known since about 1950. They are used on a very wide scale in memory systems of electronic computers, also in minor quantities for high-speed devices where the internal directional change of domain alignment functions in a manner comparable to the moving parts of a mechanical switch.

This application is a continuation in part of U.S. application Serial No. 442,534, filed July 12, 1954, which in turn is a continuation in part of U.S. application Serial No. 270,351, filed February 7, 1952 (now abandoned), U.S. application Serial No. 253,779, filed October 30, 1951 (now abandoned), and U.S. application Serial No. 67,752, filed December 28, 1948 (now abandoned).

The said U.S. application Serial No. 442,534 relates to  $MgO$ — $MnO$ — $Fe_2O_3$  ferrite compositions which show square hysteresis loops. These compositions may consist entirely of the components  $MgO$ ,  $MnO$  and  $Fe_2O_3$ , the components being present in the following proportions:

|           | Mole percent |
|-----------|--------------|
| $MgO$     | 8 to 55      |
| $MnO$     | 4 to 67      |
| $Fe_2O_3$ | 25 to 47.5   |

Bodies used for memory cores are generally within a somewhat narrower range as follows:

|           | Mole percent |
|-----------|--------------|
| $MgO$     | 25 to 40     |
| $MnO$     | 15 to 30     |
| $Fe_2O_3$ | 38 to 43     |

This is substantially the composition which was disclosed in U.S. application No. 253,779.

More recently square loop ferrites are allegedly found in other systems also such as in the lithium nickel ferrite system (Belgium 534,271), lithium copper ferrite system (Belgium 534,272), the nickel-magnesium-zinc ferrite system (Belgium 534,276 and 535,198), the copper nickel ferrite system (Belgium 534,277), the copper manganese ferrite system (Belgium 534,279), the cobalt manganese ferrite system (Belgium 534,757), the nickel manganese magnesium ferrite system (Belgium 535,200). To obtain the square loop properties, the proportions of the various components are within certain critical ranges.

This invention differs from said prior applications of which this application is a continuation-in-part in that the magnesium component of the  $MgO$ — $MnO$ — $Fe_2O_3$  system is replaced by a mixture of at least two oxides, preferably by a mixture of three.

The drawing shows a triaxial diagram wherein the proportions are in mole percent.

The invention can be described most accurately by reference to the triaxial diagram of the drawing, however, since there are more than three constituents, one of the triaxial coordinates represents a number of oxides instead of only one. It is the former  $MgO$  parameter which now represents several bivalent oxides; symbolized

as MO. One feature of the invention relates to the compositions defined by a certain triaxial area. This area reaches into a section of the triaxial diagram which previously was not considered to belong to the true "square-loop area" of the system (so long as this system was confined to the three oxides  $MgO$ — $MnO$ — $Fe_2O_3$ ). The area now is defined by the following mole percentage boundaries:

|    |                   |
|----|-------------------|
| 10 | 4—25 MO           |
|    | 27.5—66 MnO       |
|    | 30—47.5 $Fe_2O_3$ |

In the triaxial diagram three sides of the area follow straight percentage lines: the 4% MO line, the 25% MO line, and the 47.5%  $Fe_2O_3$  line. The fourth side follows a curved line connecting the 4 MO, 66 MnO, 30  $Fe_2O_3$  point with the 25 MO, 42 MnO, 33  $Fe_2O_3$  point.

Another feature of the invention is the variety of metal oxides representing MO. They are the oxides of magnesium, calcium, zinc, and copper.

A third feature of the invention is the particular importance of a minimum amount of magnesia of 2 mole percent, which has to be present in any of the compositions, while the other "MO" components may be present in various proportions adding up to the limit of 25 mole percent. The minimum limitation of 4 mole percent of MO means that the body contains 2 mole percent  $MgO$  and 2 mole percent of any or several of the other oxides. Except for the boundary line of 4 mole percent MO,  $MgO$  is always a minor constituent as compared with the sum of the other MO components.

A fourth feature of the invention is the specific way of firing these bodies. As the examples show, a water-vapor protective-gas firing at temperatures up to 2500° F., preferably in the vicinity of 2400° F. may be used; in other cases more advantageous properties may be obtained if the materials are fired first in air and subsequently heat-treated ("corrected") in a water-vapor atmosphere. Other neutral gases may be applied likewise.

It of course is not irrelevant which of the MO constituents at variance will be used and combined in any particular case. Depending on the properties desired different mixtures will be added for the MO component. The  $MgO$ , as is well known, enhances the sharpness of the hysteresis-loop corners;  $CuO$  acts as a flux, reduces the firing temperature, and promotes the density of the body;  $CaO$  reduces the coercive force without markedly reducing the Curie temperature, and  $ZnO$  increases saturation flux density. (In higher amounts the latter reduces the Curie temperature and impairs the rectangularity.)

The drawing is a triaxial diagram containing an outlined area which includes all the compositions of the invention.

The following examples show a variety of combinations without of course limiting the possibilities to any certain proportions. Saturation, remanence, coercive force, initial permeability and maximum permeability are indicated in every case. In some cases the ratio of remanence to saturation  $B_r/B_s$  appears comparatively low—between 0.7 and 0.8—because saturation was measured at the relatively high magnetizing field strength of 25 oersteds. Operating field strengths for optimum rectangular loop performance are usually very much lower corresponding to a  $B_r/B_s$  ratio just below or above 0.9.

### Example 1

|           | Mole percent |
|-----------|--------------|
| 70 MO     | 20           |
| MnO       | 47           |
| $Fe_2O_3$ | 33           |

MO consists of:

9.6 mole percent MgO  
2.6 mole percent CaO  
7.8 mole percent ZnO

The body is made by wet milling and mixing of the proper amounts of MgO (or  $MgCO_3$ ),  $CaCO_3$ , ZnO, MnO (or  $MnCO_3$ ) and  $Fe_2O_3$ . The dried mixture is calcined at about  $1700^{\circ} F$ , reground, and dried and granulated. Pressed parts were fired, in air at  $2460^{\circ} F$ , and subsequently refired in water vapor at  $2100^{\circ} F$ . 10

The main properties of ring-shaped cores are:

$B_s=2500$  gausses  
 $B_r=2100$  gausses  
 $H_c=0.22$  oersted  
 $\mu_0=100$   
 $\mu_{max}=4400$

Loop corners are well developed.

*Example 2*

The mole ratio as to the three components MO, MnO, 20 and  $Fe_2O_3$  is the same as that of Example 1.

MO consists of:

9.6 mole percent MgO  
2.6 mole percent CuO  
7.8 mole percent ZnO

Processing is the same as described before except that calcium is replaced by copper. Copper oxide or basic copper carbonate may serve as raw material.

The properties of the fired body are:

$B_s=2400$  gausses  
 $B_r=1700$  gausses  
 $H_c=0.24$  oersted  
 $\mu_0=63$   
 $\mu_{max}=3300$

Corners are well developed.

The replacing of CaO by CuO results in a slightly widened loop.

*Example 3*

Mole percent 40

MO ----- 20  
MnO ----- 38  
 $Fe_2O_3$  ----- 42

MO consists of:

9.6 mole percent MgO  
2.6 mole percent CaO  
7.8 mole percent ZnO

Processing is the same as described in Example 1.

The properties of the fired body are:

$B_s=3100$  gausses  
 $B_r=2200$  gausses  
 $H_c=0.3$  oersted  
 $\mu_0=175$   
 $\mu_{max}=4700$

Corners are quite distinct even for small magnetizing fields.

*Example 4*

The mole ratio of the three components MO, MnO, 60 and  $Fe_2O_3$  is the same as in Example 3, but MO consists of:

9.6 mole percent MgO  
2.6 mole percent CuO  
7.8 mole percent ZnO

Processing is the same as described in Example 3 except that calcium is replaced by copper.

The properties of ring samples fired in air at  $2410^{\circ} F$ , and refired in a water-vapor atmosphere at  $2100^{\circ} F$ , are:

$B_s=3200$  gausses  
 $B_r=2700$  gausses  
 $H_c=0.3$  oersted  
 $\mu_0=120$   
 $\mu_{max}=6000$

70

75

75

75

75

Corners are very well developed. The loop shape is excellent.

*Example 5*

|                 | Mole percent |
|-----------------|--------------|
| MO -----        | 5            |
| MnO -----       | 62           |
| $Fe_2O_3$ ----- | 33           |

MO consists of:

2 mole percent MgO  
1 mole percent CaO  
2 mole percent ZnO

Processing is the same as described in Examples 1 and 3. The properties of the body fired in air at  $2460^{\circ} F$ , and refired in water-vapor at  $2100^{\circ} F$ , are as follows:

$B_s=2300$  gausses  
 $B_r=1700$  gausses  
 $H_c=0.4$  oersted  
 $\mu_0=77$   
 $\mu_{max}=2400$

Compared with the previous examples this body displays a fairly low maximum permeability.

*Example 6*

The mole ratio of the three components MO, MnO, and  $Fe_2O_3$  is the same as in Example 5, but MO consists of:

2 mole percent MgO  
1 mole percent CuO  
2 mole percent ZnO

Processing is the same as described in Examples 1, 3, and 5 except that calcium is replaced by copper. The properties of ring samples fired in water vapor at  $2400^{\circ} F$ , are:

$B_s=2300$  gausses  
 $B_r=1800$  gausses  
 $H_c=0.6$  oersted  
 $\mu_0=80$   
 $\mu_{max}=6600$

Examples 5 and 6 demonstrate the effect of an extremely high manganese percentage. (Situated in the corner of the area Examples 5 and 6 do not represent the most favorable combination of oxides.) Example 6 shows a remarkably high maximum permeability indicating the effect of copper oxide as a fluxing agent.

*Example 7*

|                 | Mole percent |
|-----------------|--------------|
| MO -----        | 5.0          |
| MnO -----       | 47.5         |
| $Fe_2O_3$ ----- | 47.5         |

MO consists of:

2 mole percent MgO  
1 mole percent CaO  
2 mole percent ZnO

Processing is the same as described in Examples 1, 3 and 5.

The properties measured on ring samples are listed below:

$B_s=3200$  gausses  
 $B_r=2500$  gausses  
 $H_c=0.5$  oersted  
 $\mu_0=220$   
 $\mu_{max}=2600$

The body represents a less favorable point being situated on the 47.5 mole percent iron oxide boundary line.

*Example 8*

|                 | Mole percent |
|-----------------|--------------|
| MO -----        | 15           |
| MnO -----       | 48           |
| $Fe_2O_3$ ----- | 37           |

MO consists of:

7 mole percent MgO  
2 mole percent CaO  
6 mole percent ZnO

Processing is the same as indicated for the preceding formulae.

The properties after a first fire at 2410° F. and a water-vapor treatment at 2150° F. are measured as follows:

$B_s = 2800$  gauss  
 $B_r = 2150$  gauss  
 $H_c = 0.3$  oersted  
 $\mu_0 = 123$   
 $\mu_{max} = 3600$

Corners: well developed.

#### Example 9

The mole ratio of the three components MO, MnO, and  $Fe_2O_3$  is the same as in Example 8, but MO consists of:

7.0 mole percent MgO  
2.0 mole percent CuO  
6.0 mole percent ZnO

Processing is the same as described in the preceding examples.

The properties after firing at 2535° F. in nitrogen are represented by the following values:

$B_s = 2900$  gauss  
 $B_r = 2230$  gauss  
 $H_c = 0.5$  oersted  
 $\mu_0 = 120$   
 $\mu_{max} = 2770$

Corners: Sharp.

Bodies 8 and 9 are in the center of the area and show good over-all properties.

#### Example 10

##### Mole percent

|           |       |    |
|-----------|-------|----|
| MO        | ----- | 10 |
| MnO       | ----- | 52 |
| $Fe_2O_3$ | ----- | 38 |

MO consists of:

4.0 mole percent MgO  
1.5 mole percent CaO  
4.5 mole percent ZnO

Processing follows the pattern as outlined above.

The material may be fired either in one step or in two steps leading approximately to the same values, which are:

$B_s = 2900$  gauss  
 $B_r = 2050$  gauss  
 $H_c = 0.35$  oersted  
 $\mu_0 = 125$   
 $\mu_{max} = 2900$

Corners: Well developed.

To facilitate the survey of the examples, all of them are compiled in the following table:

| Example | MO | MgO | CaO   | CuO   | ZnO | CdO   | MnO  | $Fe_2O_3$ |
|---------|----|-----|-------|-------|-----|-------|------|-----------|
| 1       | 20 | 9.6 | 2.6   | ----- | 7.8 | ----- | 47   | 33        |
| 2       | 20 | 9.6 | ----- | 2.6   | 7.8 | ----- | 47   | 33        |
| 3       | 20 | 9.6 | 2.6   | ----- | 7.8 | ----- | 38   | 42        |
| 4       | 20 | 9.6 | ----- | 2.6   | 7.8 | ----- | 38   | 42        |
| 5       | 5  | 2.0 | 1.0   | ----- | 2.0 | ----- | 62   | 33        |
| 6       | 5  | 2.0 | ----- | 1.0   | 2.0 | ----- | 62   | 33        |
| 7       | 5  | 2.0 | 1.0   | ----- | 2.0 | ----- | 47.5 | 47.5      |
| 8       | 15 | 7.0 | 2.0   | ----- | 6.0 | ----- | 48   | 37        |
| 9       | 15 | 7.0 | ----- | 2.0   | 6.0 | ----- | 48   | 37        |
| 10      | 10 | 4.0 | 1.5   | ----- | 4.5 | ----- | 52   | 38        |

I claim:

1. A molded ferrite body displaying a substantially rectangular hysteresis loop consisting essentially of manganese oxide, ferric oxide and at least three additional bivalent oxides (MO) consisting of  $ZnO$ ,  $MgO$  and at least one MO selected from the group consisting of  $CaO$  and  $CuO$ ;

5 said manganese oxide consisting of 27.5-66 mol percent of the composition;

10 said ferric oxide consisting of 30-47.5 mol percent of the composition;

said  $ZnO$  consisting of at least 1 mol percent of the composition;

15 said  $MgO$  consisting of at least 2 mol percent of the composition and when over 2 mol percent being less than the sum of the mol percentages of the  $CaO$ ,  $CuO$  and  $ZnO$  components;

said ferrite containing at least 1 mol percent of the bivalent oxide selected from the group consisting of  $CaO$  and  $CuO$ ;

20 the total proportion of the  $MgO$ ,  $ZnO$ ,  $CaO$  and  $CuO$  components being 4-25 mol percent of the composition.

25 The ferrite as defined in claim 1 wherein said MO constituents comprise about 20 mol percent of the composition and consist of about 9.6 mol percent of  $MgO$ , about 8 mol percent of  $ZnO$  and an oxide selected from the group consisting of  $CaO$  and  $CuO$  in an amount approximately equal to 20 mol percent less the total mol percent of  $MgO$  and  $ZnO$ .

30 3. The ferrite as defined in claim 1 wherein said MO constituents comprise about 2 mol percent of  $MgO$ , 2 mol percent of  $ZnO$  and about 1 mol percent of an oxide selected from the group consisting of  $CaO$  and  $CuO$ .

4. The ferrite as defined in claim 1, wherein said MO constituents comprise about 15 mol percent of the composition and consist of about 7 mol percent of  $MgO$ , 6 mol percent of  $ZnO$  and about 2 mol percent of an oxide selected from the group consisting of  $CaO$  and  $CuO$ .

5. The ferrite as defined in claim 1 wherein said MO constituents comprise about 10 mol percent of the composition and consist of about 4 mol percent  $MgO$ , 1.5 mol percent  $CaO$  and 4.5 mol percent of  $ZnO$ .

#### References Cited in the file of this patent

##### UNITED STATES PATENTS

|           |                         |                |
|-----------|-------------------------|----------------|
| 1,997,193 | Kato et al. -----       | Apr. 9, 1935   |
| 2,452,529 | Snoek -----             | Oct. 26, 1948  |
| 2,452,530 | Snoek -----             | Oct. 26, 1948  |
| 2,452,531 | Snoek -----             | Oct. 26, 1948  |
| 2,535,025 | Albers-Schoenberg ----- | Dec. 26, 1950  |
| 2,551,711 | Snoek et al. -----      | May 8, 1951    |
| 2,565,058 | Albers-Schoenberg ----- | Aug. 21, 1951  |
| 2,565,111 | Albers-Schoenberg ----- | Aug. 21, 1951  |
| 2,565,861 | Leverenz et al. -----   | Aug. 28, 1951  |
| 2,568,881 | Albers-Schoenberg ----- | Sept. 25, 1951 |
| 2,640,813 | Berge -----             | June 2, 1953   |
| 2,715,109 | Albers-Schoenberg ----- | Aug. 9, 1955   |

#### OTHER REFERENCES

Physic III, June 1936, pp. 463-483.  
New Developments in Ferromagnetic Materials by Snoek, pp. 69 and 91, pub. by Elsevier Pub. Co. Inc. 65 (1947), N.Y.

UNITED STATES PATENT OFFICE  
CERTIFICATE OF CORRECTION

Patent No. 2,981,690

April 25, 1961

Ernst Albers-Schoenberg

It is hereby certified that error appears in the above numbered patent requiring correction and that the said Letters Patent should read as corrected below.

for In the drawing, lower right-hand portion of the figure,

|                 |                 |
|-----------------|-----------------|
| EXAMPLE 9 & 10  | EXAMPLE 8 & 9   |
| EXAMPLE 11 & 12 | read EXAMPLE 10 |
| EXAMPLE 7 & 8   | EXAMPLE 7       |

Signed and sealed this 7th day of November 1961.

(SEAL)

Attest:

ERNEST W. SWIDER

Attesting Officer

DAVID L. LADD

Commissioner of Patents

USCOMM-DC